

## UNITED STATES PATENT OFFICE

2,267,219

METHOD OF ELECTRICALLY TREATING  
METAL

Robert F. Renkin, Sharon, Pa., assignor of one-half to Henry A. Roemer, Pittsburgh, Pa.

No Drawing. Application January 23, 1940,  
Serial No. 315,186

7 Claims. (Cl. 205—21)

The invention relates generally to the cleaning of metal products, and more particularly to the cleaning or cleaning and coating of metal products with a relatively soft metal.

In the manufacture of relatively small gauge metal products, such as sheets, stripsheets, strips and wire, a number of successive reductions by rolling or drawing operations is required before the metal product is brought down to the desired gauge or thickness. Such cold working or reducing operations greatly diminish the ductility and workability of the metal product, so that at frequent intervals during the reducing operations the metal product must be subjected to annealing treatments to restore its ductility, followed by the usual acid pickling to remove any scale.

In making small gauge wire, after the wire has been drawn down to say 12 gauge by the preliminary drawing operations, it is in the form of extremely long strands so that in order to be handled economically and efficiently it is pickled, fluxed, and coated in coils prior to the last series of drawing operations.

However, when coils having many turns of wire are dipped in a pickling and then in a coating bath, it is an expensive and messy procedure, and where the wire is required to be coated with a relatively soft metal, it is very difficult if not impossible to obtain a uniform and adherent coating, because the turns of wire stick together in many places with the result that an uneven coating is produced.

Where steel having a very low carbon content is galvanized, as for example steel telephone wire, by passing the wire from the pickling bath into the spelter pot, the galvanized coating is not sufficiently ductile or adherent to meet certain tests required of such wire, and one method of satisfactorily galvanizing such wire is fully set forth in my copending application Serial No. 309,224, filed December 14, 1939, and entitled Method of coating metal. Such method includes subjecting the wire to a dry pickling treatment, then passing it through a special fluxing bath, and passing it into the galvanizing bath.

In the manufacture of certain metal products, as for example, stainless steel wire, it has been found expedient to coat the wire with a soft metal such as lead prior to the drawing operations, the lead acting as a lubricant during the drawing operations. Present practice in making stainless steel wire preferably includes passing hot rolled stainless steel rods through an acid etching pickle, fluxing, lead coating, and then drawing the wire down as far as possible or until

the wire becomes so brittle as to require further annealing. The stainless steel wire is then passed through an acid wash to remove the remaining lead coating, and is again annealed, pickled, fluxed, and lead coated in preparation for another series of drawing operations.

After the wire has been drawn down to say 12 gauge and annealed, the stainless steel wire must be given another etching pickle treatment, preferably in hydrochloric acid, to produce an etched surface on the wire before a lead coating can be made to adhere thereto sufficiently to act as a lubricant during subsequent drawing operations.

This etching pickle treatment causes a substantial loss of metal. In making stainless steel wire according to conventional practice, it has been found that not only are the etching and lead coating steps expensive, but the lead coating obtainable is uneven and non-adherent to the extent that a minimum number of subsequent drawing operations can be made on the wire. For example, with stainless steel wire of the order of 12½ gauge, .099" diameter, it has not been possible with conventional practice to perform more than three reductions, bringing the wire down to about .050" diameter, without reannealing.

I have discovered that the usual acid pickling treatment can be eliminated by passing the metal product, after an annealing treatment, through an electrolyzed flux wherein the metal product is made the anode, and that the metal product can then be passed directly into the metal coating bath to obtain a uniform and very adherent coating.

In applying this discovery and invention to the making of stainless steel wire, even though the wire may be semi-oxidized or bright annealed after the preliminary drawing operations, I have found that by passing the wire through an electrolyzed flux and making the wire the anode, the etching pickle step required in conventional practice can be eliminated and the wire passed directly from the flux into a molten lead bath to produce a uniform lead coating thereon.

Moreover, stainless steel wire made according to my novel method is capable of being reduced by an increased number of successive drawing operations, without reannealing, to produce a very small gauge wire product.

It is a general object of the present invention to provide a novel method of cleaning metal products by electrically treating the same.

A specific object of the present invention is to provide a novel method of producing a uniform

and adherent soft metal coating on a metal product without first pickling the metal product.

Another specific object of the present invention is to provide a novel method of uniformly coating annealed stainless steel wire with a soft lubricant without first pickling the wire.

Another object is to provide a novel method of producing small gauge steel wire with a minimum number of annealing treatments.

Another object is to provide a novel method of uniformly coating metal with lead prior to reducing or drawing the metal, whereby an increased number of drawing operations can be performed without annealing.

A still further object is to provide a novel method of cleaning and coating metal, which method produces an improved product with a minimum amount of handling and at a minimum cost.

These objects, together with others which will appear from the following detailed description of the invention, are accomplished by the method steps, and the combinations and sub-combinations thereof, which are hereinafter set forth in detail and defined in the appended claims.

By way of example, the invention will be described herein as applied to the manufacture of steel wire, but it is to be understood that, within the scope of the appended claims, the invention is applicable to the making of other ordinary steel products, such as sheets, strips, strip sheets, etc.; as well as to the manufacture of similar products of other metals.

In carrying out my novel method in the manufacture of small gauge stainless steel wire, I start with wire which preferably has been drawn down or reduced to some extent according to conventional practice. This preliminary reducing treatment may include pickling hot rolled stainless steel rods, fluxing and lead coating them, and then subjecting them to successive drawing operations, between which additional annealing, fluxing and pickling steps are interposed as and when required.

After the stainless steel wire has been thus reduced to say about 12 or 12½ gauge, it is coiled and annealed but not pickled before treating it according to my novel method. The gauge of the wire upon which I begin my novel treatment may vary according to the capacity of the equipment being used, and I mention 12 or 12½ gauge merely as an example.

The wire coils to be treated by my novel method may have been annealed so as to produce an oxidized or semi-oxidized surface on the wire, or they may have been bright annealed in an inert atmosphere such as ammonia gas. The wire is first passed through a separate fluxing bath of more or less ordinary composition, preferably by placing the coils on suitable pay off reels and feeding the wire strands continuously through the fluxing bath.

I prefer to use a flux solution having the following composition, although the composition of the flux may be varied considerably and still give satisfactory results.

#### Parts

|                                    |   |
|------------------------------------|---|
| Zinc chloride (liquid) (by volume) | 1 |
| Zinc ammonium chloride (crystals)  | 2 |
| Sal ammoniac                       | 1 |
| Water                              | 1 |

which gives a very saturated solution having a Baumé reading of about 45°, operating at 175°-200° F.

A very important feature of the invention is

that the flux is constantly electrolyzed with the wire acting as the anode and preferably the flux tank acting as the cathode. This may be done by connecting the positive terminal from a power

source to one of the usual wire holddown rolls immersed in the flux, thus making the wire the anode, and by connecting the other terminal from the power source to a convenient place on the flux tank wall, thus making the tank the cathode.

The amount of current and fluxing time required will vary according to the size of the apparatus used and the various operating conditions, but I have successfully treated 12½ gauge stainless steel wire using a direct current of 7½ to 15 volts with 20 to 40 amperes, and immersing the wire in the flux from 5 to 10 seconds.

From the fluxing bath, the wire is led directly into and through a separate bath of molten lead formed of ordinary or commercial lead maintained at approximately 620° to 670° F., after which the wire is ready for further drawing operations.

The reaction of the electrolyzed flux using the wire as the anode is difficult to explain, but apparently a cleaning or deplating of the wire surface is effected, and a uniform flux film is deposited on the wire as it leaves the fluxing bath. At any rate when the wire is passed from the fluxing bath directly into a separate bath of molten commercial lead, a very uniform adherent lead coating is obtained on the wire.

In cleaning and coating 12½ gauge, .099" diameter stainless steel wire according to this method, I have been able to then pass the wire through five successive drawing operations without reannealing, to satisfactorily produce wire of .037" diameter.

The step by step reductions for these five drawing steps were as follows:

|             |                |
|-------------|----------------|
| First draw  | .099" to .082" |
| Second draw | .082" to .069" |
| Third draw  | .069" to .053" |
| Fourth draw | .053" to .044" |
| Fifth draw  | .044" to .037" |

With prior conventional practice wherein 12½ gauge stainless steel wire was annealed, pickled in acid, fluxed, and then lead coated, great difficulty was experienced in obtaining a lead coating which was sufficiently adherent, and it was practically impossible to produce a uniform lead coating, with the result that the coated wire could not be given more than three draws, reducing it to about .050" diameter before reannealing.

Accordingly, my invention provides a novel and improved method of cleaning and coating stainless steel wire without the usual pickling, making possible an increased number of drawing operations to produce wire of smaller gauges than has heretofore been possible, without reannealing.

When it is desired to galvanize metal products on which it is difficult to obtain a uniform and adherent coating, as for example low carbon steel telephone wire, the wire can be taken from the annealing furnace, or from the dry pickling furnace described in my copending application Serial No. 309,224, and passed through the electrolyzed flux containing preferably zinc chloride, zinc ammonium chloride and sal ammoniac as set forth herein, with the wire acting as the anode.

By then passing the wire directly through a separate galvanizing bath, a galvanized coating is produced on the wire, which coating is suffi-

ciently ductile and adherent to withstand the severest tests required of it, as for instance, bending the coated wire about its own diameter.

I claim:

1. A method of cleaning and coating metal, which includes annealing the metal, passing the metal through a separate flux solution containing zinc chloride electrolyzed by passing an electric current through the flux with the metal as the anode, and then passing the metal directly 10 into a separate molten coating bath.

2. In a method of cleaning and coating steel, the steps of passing the steel through a separate flux solution containing zinc chloride electrolyzed by passing electric current through the flux with the steel acting as the anode, and then passing the steel directly into a separate molten lead coating bath.

3. A method of cleaning and coating stainless steel which includes annealing the steel, passing the steel through a separate flux solution containing zinc chloride electrolyzed by passing electric current through the flux with the steel acting as the anode, and then passing the steel directly into a separate bath of molten commercial lead.

4. A method of cleaning and coating stainless steel wire for cold drawing, which includes annealing the wire, passing the steel through a separate flux solution containing zinc chloride, zinc ammonium chloride and sal ammoniac, electrolyzing the flux during the passage of the wire therethrough by passing an electric current through the flux with the wire acting as the

anode, and then passing the wire directly into a separate bath of molten lead.

5. In a method of treating metal, the steps of annealing the metal, and then cleaning and fluxing the metal by moving the metal through a separate flux solution containing zinc chloride, zinc ammonium chloride and sal ammoniac, and electrolyzing the flux during the passage of the metal therethrough by passing an electric current through the flux with the metal acting as the anode.

15 6. A method of reducing stainless steel wire which includes annealing the wire, passing the wire through a separate flux solution containing zinc chloride, electrolyzing the flux during the passage of the wire therethrough by passing an electric current through the flux with the wire acting as the anode, then passing the wire through a separate bath of molten lead, and then 20 subjecting the wire to successive drawing operations to 60 to 65 per cent reduction, without re-annealing the wire.

25 7. A method of reducing metal which includes annealing the metal, passing the metal through a separate flux solution containing zinc chloride, electrolyzing the flux during the passage of the metal therethrough by passing an electric current through the flux with the metal acting as the anode, then passing the metal through a 30 separate molten lead coating bath, and then subjecting the metal to successive cold working operations.

ROBERT F. RENKIN.